

United States Patent [19]  
Vause

[11] 3,818,558  
[45] June 25, 1974

[54] **METHOD OF MAKING LAMP CAP CONNECTIONS USING SUPERPLASTIC ALLOY**

3,713,207 1/1973 Ruckle et al. .... 29/498

[75] Inventor: **Arthur Samuel Vause, London, England**

OTHER PUBLICATIONS

Hayden, H. W. et al., "Superplastic Metals," Scientific American, March 1969, pp. 28-35.

[73] Assignee: **Thorn Electrical Industries Limited, London, England**

Primary Examiner—Roy Lake  
Assistant Examiner—J. W. Davie  
Attorney, Agent, or Firm—Robert F. O'Connell,  
Dike, Bronstein, Roberts & Cushman

[22] Filed: **June 4, 1973**

[21] Appl. No.: **366,739**

[30] **Foreign Application Priority Data**

June 6, 1972 Great Britain ..... 26398/72

[52] U.S. Cl. .... **29/25.13, 29/504, 313/331**

[51] Int. Cl. .... **H01j 9/18**

[58] **Field of Search** ..... 29/25.13, 489, 484, 498,  
29/504; 313/318, 331; 339/144, 145;  
148/11.5 R

[56] **References Cited**

UNITED STATES PATENTS

2,987,696 6/1961 Rudler et al. .... 313/318 X

[57] **ABSTRACT**

Electric lamps are disclosed having lead-in wires which extend out of the lamp envelopes and are connected to external electrical terminals, the terminals including hollow metal sleeves receiving the wires and the wires being joined thereto using alloys which exhibit superplastic behaviour, the alloys being heated, without melting, and caused to flow or creep superplastically into the sleeves and around the wires.

8 Claims, 4 Drawing Figures



PATENTED JUN 25 1974

3,818,558

FIG. 1.



FIG. 2.



FIG. 3.



FIG. 4.



## METHOD OF MAKING LAMP CAP CONNECTIONS USING SUPERPLASTIC ALLOY

The present invention relates to improved lamps and particularly to improvements in lamp cap connections to lead-in conductors.

At some stage during the manufacture of an electric lamp it is necessary to make permanent electrical connections between a lamp cap or base and one or more lead-in conductors such as wires which extend into the interior of the lamp. The lead-in wire or wires may be connected to the shell of the cap, or to contact pads or to pin terminals with which the cap is provided, depending upon the form of the cap and the type of electrical socket which the lamp is intended to fit. The normal method of connecting lead-in wires to cap contacts involves soldering.

Soldering is not entirely satisfactory, however, and presents various problems both during manufacture and use, and can also impose limitations on the design of lamps and associated fittings. It can be extremely difficult to arrange that only just that quantity of solder needed to cover the lead-in wires and to form adequate connections is dispensed by automatic soldering machines. Furthermore, a flux normally has to be used when soldering. Fluxes are frequently corrosive and, when cold, may be in the form of hard, glassy substances. These characteristics of fluxes makes it relatively difficult and time consuming to maintain soldering machinery properly.

When in use, a lamp may be subjected to high temperatures which can cause softening of soldered connections. In turn, softening can lead to connections breaking and possibly to a lamp becoming soldered to the electrical socket itself. Another possible fault arising from the use of solder is that arcing between the socket and the lamp cap may arise, with consequent damage to both the socket and the lamp. The onset of arcing is encouraged by irregularities on the solder surface, and the occurrence of irregularities such as spikes of solder is difficult to prevent during automated manufacture.

The shells of lamp caps which form part of the conductive paths between the lamps and their sockets are commonly made of brass because it is easy to make soldered connections thereto. An example of such a lamp is one having an Edison screw-cap. Brass is expensive, however, and for this reason it would be preferable if aluminium could be substituted instead. Unfortunately, aluminium does not adequately lend itself to soldering in a simple and economical manner. There are many problems standing in the way of making intimate and durable electrical connections to aluminium lamps caps on high speed automated lamp-making machines.

In accordance with the present invention therefore, there is provided a method of finishing an electrical lamp which has a lead-in conductor sealed through the envelope of the lamp and terminating outside the envelope, wherein an electrical terminal is made by threading the outer end of the conductor into a hollow member which forms a well around the conductor, the lamp is inverted such that the well is uppermost, and an alloy capable of exhibiting the phenomenon of superplasticity is placed in the well and heated to a temperature, below its melting temperature, at which it behaves superplastically to cause it to flow into a compact mass

in intimate contact with the conductor. No flux is needed when carrying out the method since no melting is involved, and hence contamination of machinery and consequent difficult maintenance is avoided. Preferably, the hollow member forming the well has a re-entrant portion serving to ensure that the mass of alloy is securely retained therein. If the method is applied to a general lighting service lamp bulb, the well can be formed directly in the body of insulation contained within the shell of an Edison screw or bayonet-type lamp base. Alternatively, the well is formed by a shaped metal ferrule which is embedded in the insulation. In lamps having post or pin terminals, the well is formed by a hollow metal sleeve element.

In practice, the superplastic material is given a preliminary heat treatment involving annealing and rapid quenching, to ensure that the material is in a condition in which it will be able to exhibit superplasticity. The material is then placed in contact with the two surfaces to be joined, i.e., a lead-in conductor and the well, and is then reheated. During this reheating, the material becomes superplastic and can then flow into intimate contact with the two surfaces. Thereafter, the temperature is reduced to ambient and it is found that a rigid joint is obtained possessing good electrical characteristics.

It is preferred to use an alloy consisting of 22 percent Aluminium and 78 percent Zinc for the bonding material. This alloy can be obtained from the Imperial Smelting Corporation (N.S.C.) Limited, Avonmouth and is known by the terms "S.P.Z." and "Prestal." The alloy exhibits free flowing superplastics behaviour when its temperature is in the range of 250° to 275°C. After cooling from this temperature range, the alloy can only recover superplasticity if heated to a somewhat higher temperature range and then quenched rapidly. The higher temperature range is approximately 275° to 375°C. Accordingly, if a lamp embodying the invention is operated normally in a hot environment, the joint is not adversely affected. The reason is that once the material has been cooled from its superplastic condition during manufacture, it loses its superplasticity and this is not normally regained later under the usual heating conditions which the lamp in service undergoes. Superplasticity can only return after the material has been heated to a critical temperature range and then rapidly quenched - a thermal treatment which is not duplicated in service.

It has been found that the above alloy is capable of making strong, durable bonds to clean aluminium as well as brass. Aluminium is the preferred lamp cap material not only on the grounds of cost, but also because aluminium and the above alloy have similar thermal coefficients of expansion.

The invention will now be described by way of example with reference to the accompanying drawings, in which:

FIG. 1 is an elevational view, with parts in cross section, of a general lighting service lamp bulb,

FIG. 2 is a partial cross sectional view of a bayonet type lamp cap,

FIG. 3 is a fractional view of a fluorescent lamp with part shown in cross section, and

FIG. 4 is a cross section through a pin-type lamp terminal.

The invention is equally applicable to the manufacture of incandescent lamps and arc discharge lamps. A

selection of lamps and lamp end fittings embodying the invention are shown in the drawings.

In FIG. 1, an incandescent filament lamp 10 is shown, having a filament 11 within an enclosing envelope 12. The filament 11 is supported upon conductors 13, 13a embedded in a neck 14 which is sealed to an end portion of the envelope 12. The conductors 13, 13a serve as lead-in wires for connecting the filament electrically to a supply, and are electrically connected to the two poles of an Edison screw lamp base 15. The base 15 includes a metallic shell 16, e.g. of brass or aluminium, which is bonded to the end portion of the envelope 12 with cement 17. In this instance, one lead-in conductor, 13a is electrically connected to the shell 16 by being trapped between the upper rim thereof and the outside of the envelope 12. The other lead-in conductor 13 is electrically connected to a metal ferrule 18, e.g. of brass or aluminium, which is centred in the end of the lamp base 15. The ferrule 18 can be an integral part of a sole plate. The electrical connection is way of a mass of superplastic alloy 19 filling the ferrule 18, the conductor 13 being embedded in the alloy 19. Instead of connecting the conductor 13a to the shell 16 as shown, it could be connected by means of superplastic alloy. In that case, the shell 16 would be provided with a cupped opening - similar in shape to the ferrule 18. The conductor would then be threaded into the opening and secured thereto with a mass of the superplastic alloy. The lamp cap 15 is completed by a filling of a heat-resistant insulating material 20. The material 20 can be a ceramic cement or a material such as "Vitrite", and serves to isolate the ferrule 18 electrically from the cap shell 16.

It will be appreciated that the Edison screw lamp base 15 can be applied to other types of lamp, such as high performance, metal halide discharge lamps.

An alternative lamp base 25 is shown in FIG. 2. This base 25 is a bayonet type, having a brass or aluminium shell 26 and bayonet studs 27. Each of the two lead-in conductors 13 extends through the interior of the shell 26 and terminates inside a ferrule 28 at the outer end of the base 25. The ferrule 28 is filled with superplastic alloy 29 and the conductor 13 is embedded therein. As shown, the surface 30 of the alloy 29 presents a smooth convex bulge for making contact with an associated sprung terminal inside a bayonet lamp socket. It will be realised that the second lead-in conductor and alloy-filled ferrule are located behind those shown in the sectional view of FIG. 2. The conductors 13, ferrules 28 and shell 26 are insulated from one another by a filling of temperature resistant insulating material 31.

A discharge lamp embodying the invention is shown in FIG. 3. The lamp 33 can be a metal halide arc discharge lamp or a fluorescent lamp. The exact form of the discharge electrode 34 will depend upon the design of the lamp, as is known, and does not form part of this invention. In this instance, the electrode 34 takes the form of a heater filament and is coated with an electron-emissive compound. It is supported on lead-in conductors 35 which are sealed through the end of an envelope 36 and enter a base or cap 37. The cap 37 has a shell 38 and a pair of pin terminals 38 suitably secured thereto and insulated from one another. Each pin terminal consists of a hollow sleeve within which one of the conductors 35 terminates. The sleeve is filled with superplastic alloy 40 which surrounds the conductor 35 and joins it mechanically and electrically to the

sleeve. To assist entry of the alloy 40 into the sleeves during manufacture, the free, lower ends of the sleeves have internally-flared mouths as shown.

A rather differently formed pin or post terminal 42 is shown in FIG. 4. Such a terminal is suitable for use in automobile lamps, projector lamps and high power incandescent or discharge lamps. The lead-in conductor 44 enters and terminates in a hollow metal sleeve 45, the interior of which is filled with superplastic alloy 46. As shown, the wall of the sleeve 45 has a dimple forming a re-entrant portion 47. This re-entrant portion is similar to the concavely-shaped ferrules 18,28 shown in FIGS. 1 and 2, and likewise serves to key the alloy firmly inside the sleeve. The strength of the joint is enhanced by forming a bend, kink or similar irregularity 49 at the end of the conductor 44.

Manufacture of lamps embodying the invention is as follows. The filaments or discharge electrodes are attached to lead-in conductors and are then sealed into their lamp envelopes using standard techniques. Gas-filling and exhaustion of the envelopes likewise is carried out using well known techniques. The outer ends of the lead-in conductors are then threaded through hollow metal elements 18,28, 39,45 which are preferably so shaped as to provide mechanical keying of the superplastic alloy which is subsequently admitted into the hollow metal elements. The inner ends of these elements 18,28, 39,45 are preferably closed, either by Vitrite 20, as in FIGS. 1 and 2, or by being sealed directly into the envelope. The partially-finished lamps are then inverted from their positions shown in the accompanying drawings, and the superplastic alloy is then inserted into the said hollow elements 18,28,39,45 which form wells surrounding the conductors. The alloy is introduced in the form of wire, strip or pellets, and sufficient is used to ensure that it just fills or slightly overfills the space around the lead-in conductor. The hollow element and alloy are then heated to the temperature at which the alloy exhibits superplasticity, whereupon it flows or creeps into intimate contact with the conductor and the inner contour of the hollow element, thereby forming a secure joint.

The preferred alloy consists of 22 percent aluminium; 78 percent zinc. This alloy is able to exhibit superplasticity after an initial heat treatment or anneal between 275° and 375°C, followed by rapid quenching. This treatment results in a very fine-grained duplex microstructure. When the alloy is in this state, subsequent heating to 250° to 275°C (in the neighbourhood of the eutectoid transformation) results in easy viscous flow. Upon slow cooling to room temperature, e.g. in air, the microstructure coarsens with grain growth. Subsequently no superplastic behaviour is observed, unless the alloy is reheated to 275° to 375°C followed by rapid quenching.

It is found convenient to heat the alloy pellets by focussed infra-red radiation, and to press the heated alloy gently into the hollow metal element. This facilitates flowing of the alloy into the said element. Instead of pressing the alloy, one could employ suction in suitably designed lamps. The resulting joint is particularly strong, and its strength is enhanced by ensuring that the hollow element and the conductor are clean and free from grease and foreign particles.

Micrographic examination of sections through alloy-filled brass or aluminium hollow elements shows that a

very smooth, continuous and intimate interface forms between the alloy and the neighbouring surface.

Other alloys which exhibit superplasticity may be used. Alloys which flow at temperatures in the range of 200°-500°C may be used, and those which flow when heated to 250°-300°C are preferred for convenience in manufacture. Examples of suitable alloys are given in the following table.

| ALLOY               | SUPERPLASTIC TEMPERATURE OR TEMPERATURE RANGE |
|---------------------|-----------------------------------------------|
| 1. Al-33% Cu        | 445°-530°C                                    |
| 2. Al-12% Cu        | 500°C                                         |
| 3. Al-12% Si-4% Cu  | 500°C                                         |
| 4. Mg-33% Al        | 350°-400°C                                    |
| 5. Mg-30% Cu        | 450°C                                         |
| 6. Mg-23% Ni        | 450°-475°C                                    |
| 7. Mg-0.5% Zr       | 500°C                                         |
| 8. Mg-6% Zn-0.5% Zr | 270°-300°C                                    |
| 9. Zn-5% Al         | 285°C                                         |
| 10. Zn-40% Al       | 250°C                                         |

The percentages given in this specification are percentages by weight.

In some alloys, superplasticity may re-appear after cooling, upon subsequent heating. To prevent this occurring during service, the alloy should be heat-treated after it has filled the hollow element and formed the joint. Such a treatment consists of an anneal at a temperature high enough and for a duration long enough to yield a coarse grained microstructure.

Whilst the embodiments shown in FIGS. 1 and 2 have hollow metal sleeves or ferrules 18, 28 containing the alloy, the ferrules could be omitted. Then, the ceramic or Vitrite 20 would be formed with a contoured opening to form a well for containing the alloy 19, which would be in direct contact therewith. The contour of the opening should have a re-entrant to ensure that the bead of alloy is firmly held in place. In such a modification, it would also be desirable for the conductor 13 to possess an irregularity such as a lobe or kink.

I Claim:

1. In a method of making a lamp having an hermetically sealed envelope through which a lead-in conductor is sealed, the conductor terminating outside the envelope, the steps of providing the lamp with an electrical terminal wherein:

a hollow member is disposed over the outer end of said conductor to form a well therearound, the lamp being inverted with said well uppermost, an alloy capable of exhibiting the phenomenon of superplasticity is placed in said well and said alloy is heated to a temperature, below its melting temperature, at which it behaves superplastically to cause said alloy to flow into said well and form a compact mass in intimate contact with said conductor.

2. A method according to claim 1, wherein said hollow member is formed with a re-entrant portion to retain said alloy securely therein.

3. A method according to claim 1, wherein said hollow member is a metal sleeve serving as a pin terminal in the finished lamp.

4. A method according to claim 1, wherein said alloy is one which is capable of exhibiting superplastic behaviour at temperatures within the range 200° to 500°C.

5. A method according to claim 4, wherein said alloy is one which is capable of exhibiting superplastic behaviour at temperatures within the range 250° to 300°C.

6. A method according to claim 5, wherein the composition of said alloy is 22 weight percent Aluminium; 78 weight percent Zinc.

7. A method according to claim 1, wherein said alloy is caused to flow into said well under the influence of gravity and with the assistance of pressure applied to said alloy.

8. A method according to claim 1, wherein said alloy is heated by focussed infra-red radiation.

\* \* \* \* \*